

Jan. 20, 1953

H. E. SPOONER

2,625,737

METHOD OF MAKING ELECTRICAL CONTACTS

Filed Aug. 25, 1950

Fig. 1.



Fig. 2.



Fig. 4.



Fig. 3.



INVENTOR.

HOWARD E. SPOONER

BY

*Paul Chirino*  
ATTORNEY

## UNITED STATES PATENT OFFICE

2,625,737

METHOD OF MAKING ELECTRICAL  
CONTACTS

Howard E. Spooner, Attleboro, Mass., assignor to  
D. E. Makepeace Company, Attleboro, Mass., a  
corporation of Massachusetts

Application August 25, 1950, Serial No. 181,449

3 Claims. (Cl. 29—155.55)

1

This invention relates to electrical contact elements suitable for use in the making and breaking of electric circuits and to methods for manufacturing such elements.

Heretofore electric make-and-break contacts for applications such as voltage regulators, relays and the like have been formed from base metal strips with precious metal inserts or inlays or rivets which serve as the contact points. The precious metals have excellent current carrying capacities due to their low electrical resistance and they are highly resistant to tarnish and electrical erosion whereby electrical contacts formed from these metals have low contact surface resistance even with small contact pressures and they are capable of maintaining a low electrical resistance in service for long periods of operation.

The present invention provides for improvements in the methods of making contacts, and an object of this invention is to produce improved electrical contacts and to save precious metals in the manufacture thereof. Further objects and various advantages of this invention will become apparent from the following description of preferred forms, reference being made to the accompanying drawings, in which, unless otherwise indicated, corresponding elements are similarly numbered throughout the various figures. The essential characteristics are summarized in the claims.

In the drawing:

Fig. 1 is a face view of a base metal strip used in fabricating contacts embodying the invention;

Fig. 2 is a side elevation of an individual plug greatly enlarged;

Fig. 3 shows the operation of punching the plug from a laminated metal strip greatly enlarged;

Fig. 4 is a face view of the die shown in Fig. 3;

Fig. 5 is an enlarged section of a contact element drawn and cut from the strip of Fig. 1.

Referring to the drawing, there is shown in Fig. 1 a wide flat strip 10 formed of any suitable electrically conductive base metal, e. g. copper, nickel, and so forth, or alloys thereof, such for example as brass, bronze, nickel-silver, etc. The strip 10 is run through a punch press which punches out a series of bores 11, the location and number of the bores being dependent upon the shape and construction of the electrical contact element that is to be manufactured. The contact element which was chosen for illustration purposes has three precious metal contact points and accordingly there

are three bores 11 punched in the strip 10 for each contact element to be manufactured.

A series of locating or centering holes 12 is also punched in the strip 10 in a line parallel to an edge of the metal strip, the centering holes being spaced apart by a distance equal to the length of strip needed to form one contact element.

In Fig. 2, there is shown a flat laminated metal plug 13, the shape and size of which is such that it will press fit into a bore 11. The thickness of the plug 13 preferably approximates that of the metal strip 10. The plug 13 is punched out from a metal strip 14 (Fig. 3) having a film or layer *a* of solder on the bottom surface thereof. The strip 14 is preferably formed from a compound metal stock having a relatively thick base or foundation *b* of an inexpensive metal, such as, for example, that from which the metal strip 10 is formed, and a thin layer *c* of a precious metal such as gold, silver, platinum, palladium and alloys of these metals. The layer *c* may be electroplated on the surface of the foundation *b*, or the layers of metal may be integrally bonded together by direct weld with the application of heat and pressure, or by brazing or soldering, all as is well known to those skilled in the art. Obviously, of course, the strip 14 may consist entirely of precious metal with a film *a* of solder on one of its surfaces.

The plug 13, herein shown as a disc, is punched out from the metal strip 14 by passing the strip between a die 16 and punch 17, with the solder face *a* of the strip towards the die and its precious metal face towards the punch. The die 16 is provided with serrations 18 around the rim of the die hole 19 (see Fig. 4). These serrations cause the solder layer *a* to be drawn up around the sides of the disc 13 as the disc is being punched out from the strip 14, thereby forming the scalloped edge 20 of the solder layer as is shown in Fig. 2.

With the strip 10 prepared as illustrated in Fig. 1, the next step in the manufacture of the electric contacts of this invention comprises fixing the discs 13 into the bores 11. This may be accomplished by supporting the die 16 upon a base 21 and passing the flat strip 10 between the base and the die so that the discs 13 when punched from the strip 14 will pass through the die hole 19 and become seated in the bores 11 in the strip 10. In order to maintain the strip in proper relative position so that the bores 11 are aligned with the die hole 19, the die 16 is provided in its bottom surface with a recess 21

of the same depth and width as the strip 10 for carrying the strip. Fig. 3 shows the punch 17 in a position after having punched out the disc 13 and before it has seated the disc into a bore 11. A guide plate 23 for the punch 17 is pref- 5 erably mounted above the strip 14.

The assembly of the strip 10 containing the discs 13 is then heated as by passing the strip through a furnace at the liquidus temperature of the solder. Upon being heated, melted solder 10 will flow between the sides of the discs and the walls of the base metal bore 11 so that the discs become firmly bonded into the strip.

The finished contacts 25 (Fig. 5) are formed from the assembled strip by a series of stamping, 15 drawing and cutting operations, the particular sequence of these operations being immaterial for the purposes of this invention so long as projections 26 which serve as the contact points are drawn out with their precious metal layers on 20 the outer surface of the projection.

It is thus apparent that this invention provides a method for manufacturing an improved electrical contact having longer wearing properties and greater corrosion resistance exactly 25 where needed and permits of the most economical use of costly noble or precious metals or alloys of these metals, since only the very point of contact is made from these metals.

It is understood that this invention is not limited to the specific embodiments shown and described and that various deviations may be made therefrom without departing from the spirit and scope of the appended claims.

What I claim is:

1. The method of making an electrical contact from a base metal strip including at least one disc-like plug formed from a laminated stock having a precious metal top layer and a bottom layer of solder, said method comprising the steps of inserting said plug with its bottom layer facing said strip into a hole in said strip while simultaneously causing solder to be drawn up around the sides of said disc, bonding said plug at its peripheral surfaces in said hole in the strip by heating said plug and strip assembly to a temperature sufficient to cause said solder to bond the peripheral sides of said plug to the walls of said hole to form a completed base strip capable of being further worked, and thereafter forming a projection in the bonded assembly including at least said plug with its precious metal layer being projected forward to serve as the contact point.

2. The method of making an electrical contact comprising sequentially punching at least one disc from a laminated stock having a precious metal bonded to one side of a base metal foundation layer and a film of solder on the other side thereof with the solder film facing downwardly, 60

said punching step being performed by means of a die having serrations around the rim of the die opening whereby the solder is caused to be drawn up around the sides of the disc, and inserting said disc into a perforation in a second base metal strip, heating said disc while being carried in said perforation to the liquidus temperature of said solder so that the disc becomes joined to said strip at its peripheral edges, and thereafter forming a projection in said bonded assembly, the apex of said projection comprising said disc with said precious metal layer forming the outer surface of said projection whereby an electric contact is formed having the precious metal contact material only at the point where needed.

3. The method of making electrical contacts comprising bonding a precious metal layer to one surface of a first strip of an electrically conductive base metal, depositing a layer of solder on the other surface of said first strip whereby a laminated metal strip is formed, punching a series of holes in a second strip of electrically conductive base metal, positioning said first strip above said second strip with the solder layer facing towards said second strip, sequentially punching a disc from said first laminated strip by means of a die having serrations around the rim of the die opening and inserting said disc into a hole in said second strip whereby the solder is caused to be drawn up around the sides of said disc, heating said disc and second strip assembly to a temperature sufficient to cause said solder to bond the peripheral sides of said disc to the second base strip to form a completed base strip capable of being further worked, stamping a series of blank electrical contact forms from said completed base strip each of said forms including at least one of said discs, and thereafter forming projections to serve as contact points in said electrical contact forms including at least one disc with the precious metal layer of said disc on the outer surface thereof.

HOWARD E. SPOONER.

#### REFERENCES CITED

The following references are of record in the file of this patent:

#### UNITED STATES PATENTS

| Number    | Name             | Date          |
|-----------|------------------|---------------|
| 1,046,823 | McBerty          | Dec. 10, 1912 |
| 2,018,073 | Laise            | Oct. 22, 1935 |
| 2,199,240 | Gwyn, Jr.        | Apr. 30, 1940 |
| 2,216,510 | Burns            | Oct. 1, 1940  |
| 2,254,558 | Williams         | Sept. 2, 1941 |
| 2,373,861 | Van Inwagen, Jr. | Apr. 17, 1945 |
| 2,414,463 | Gunn et al.      | Jan. 21, 1947 |